

A. G. MCKENNA.  
INGOT CASTING.  
APPLICATION FILED MAY 16, 1912.

1,119,088.

Patented Dec. 1, 1914.



Witnesses

Thomas Durant  
Halbert Brown

Fig. 1.

Alexander George McKenna

By Church & Church

his Attorneys.

Inventor

# UNITED STATES PATENT OFFICE

ALEXANDER GEORGE MCKENNA, OF WASHINGTON, DISTRICT OF COLUMBIA.

## INGOT-CASTING.

1,119,088.

Specification of Letters Patent.

Patented Dec. 1, 1914.

Application filed May 16, 1912. Serial No. 697,791.

To all whom it may concern:

Be it known that I, ALEXANDER GEORGE MCKENNA, a citizen of the United States, residing at Washington, in the District of Columbia, have invented certain new and useful Improvements in Ingot-Casting; and I do hereby declare the following to be a full, clear, and exact description of the same, reference being had to the accompanying drawings, forming part of this specification, and to the figures and letters of reference marked thereon.

This invention relates to improvements in metal casting and particularly the casting of ingots of steel and similar metal.

It is well known that in casting ingots the metal in solidifying forms cavities or "pipes," and while many attempts have been made to prevent such piping or the formation of cavities or to cure the defects resulting from the formation of the same, such efforts from a practical standpoint have usually resulted in indifferent success. Because of this and the extra cost and labor, casting operations are usually carried on without serious effort to overcome the difficulty with the result that the castings and articles manufactured from the castings are defective and liable to develop flaws and break down unexpectedly at points where the metal should be solid and homogeneous.

I have discovered that a complete cure for the difficulty consists in filling the cavities or piping at the time of casting; and while the metal is still hot, with molten metal of the same or substantially the same composition as the casting, the heat of the added metal being much higher than that necessary or employed in melting the metal for the body of the casting, whereby the added metal will not only penetrate the interstices formed in the casting, but will without the use of an excess of metal supply sufficient heat to melt down any obstructions and form a homogeneous mass with the walls of the cavities or interstices by fusing the same.

With furnaces in which the steel is melted in crucibles or in a hearth through radiation from flames, it is difficult to superheat the steel sufficiently, as the container will be destroyed, but electric furnaces in which the steel may be heated to a higher degree than the walls of the container may be employed

and the metal readily heated to the desired temperature, conveniently termed super- 55 heated.

It is preferred that the metal to be supplied to the casting shall be superheated in a relatively small portable furnace made in the form of a ladle with a bottom discharge, 60 so as to avoid loss of heat during transferance and to permit of the heat being maintained to the very moment when the metal passes from the ladle to the casting.

In the drawings.—Figure 1 is a conventional section showing a ladle and ingot mold, with molten metal flowing from the former into the latter. Fig. 2 is a similar section of the ingot mold after the metal has congealed therein. Fig. 3 is a similar 70 section of a small superheating ladle. Fig. 4 is a similar section of the small superheating ladle and ingot mold showing the method of filling the pipe in the ingot.

Like letters of reference in the several figures indicate the same parts.

In practice the steel will be melted, as usual, in an open hearth or other suitable furnace from which it will be drawn into a large ladle such as A, Fig. 1 adapted to be 80 tapped from the bottom. When the slag begins to run from the furnace the large ladle is removed by a crane and a small electric furnace ladle such as B placed in position to receive a portion of the slag, sufficient to 85 cover any metal which may be subsequently poured into the ladle. A suitable quantity of the molten steel is now drawn from the large ladle into the small electric furnace ladle, and the large ladle is carried to the 90 molds (C in the drawing) and poured (Fig. 1) in the usual manner. During this operation or at the proper time current is supplied to the small ladle (an A. C. generator D being indicated in Fig. 3 of the drawing for 95 this purpose) and the metal in the small ladle is superheated. When the castings have cooled to a point where the piping has taken place or the cavities have formed (Fig. 2), the time depending upon the size of the ingots or castings, the electric furnace ladle is carried over the molds and the pipes or cavities filled with the superheated steel (as shown in Fig. 4). The superheated steel not only fills all cavities and interstices, but 105 melts down any obstructions and becomes

2  
completely homogeneous with the body of the casting.

Obviously the slag coverings for the metal in the ladles need not be employed, but are 5 desirable to conserve the heat and protect the surface of the metal during the pouring and heating operations.

With the present invention there is no excess of metal used and consequently no 10 waste. The process is economical both because of the saving of metal and because it is only necessary to superheat a relatively small percentage of the metal for making the casting.

15 Having thus described my invention, what I claim as new and desire to secure by Letters Patent of the United States, is:

1. The process of casting ingots in molds which consists in pouring the metal into the 20 mold and permitting the same to congeal, then pouring into the pipes and interstices therein molten metal sufficient in quantity to fill the pipes and interstices without excess, said molten metal being superheated to 25 a temperature sufficient to fuse the walls of

the pipes and interstices and unite therewith to form a homogeneous mass.

2. The improvement in the process of casting ingots which consists in filling the 30 pipes and interstices therein with superheated molten metal of substantially the composition of the body of the ingot.

3. The improvement in the process of casting ingots, which consists in superheating a relatively small percentage of the molten metal from which the ingot is cast and in filling the pipes and interstices in the ingot with the superheated metal. 35

4. The improvement in the process of casting ingots which consists in superheating a portion of the molten metal in a movable heater and in transferring the heater to and discharging the superheated metal therefrom directly into the pipes and interstices in the ingot. 40

ALEXANDER GEORGE MCKENNA.

Witnesses:

HARRY F. CLARK,  
WALTER ANDERSON.